

## UNITED STATES PATENT OFFICE.

RICHARD F. SPROESSIG, OF HOLTON, INDIANA.

## PROCESS FOR MAKING METAL PACKING.

No Drawing.

Application filed March 7, 1921. Serial No. 450,450.

*To all whom it may concern:*

Be it known that I, RICHARD F. SPROESSIG, a citizen of the United States, and residing at Holton, in the county of Ripley and State of Indiana, have invented a new and useful Process for Making Metal Packing, of which the following specification is a full disclosure.

My invention relates to the production of 10 metallic packing material amalgamated with a lubricant and to a metal alloy packing product of spongy constituent permeated or impregnated with a pulverulent lubricant.

An object of the invention is to provide a 15 simple and efficient method for efficiently permeating a metal alloy with a determined per cent of lubricant and forming a product more ductile and malleable for compressing and shaping into form for an article 20 of commerce or as a compound for packing purposes.

Another object of the invention is to pour the molten metal or metal alloy from a determined height into a bath of pulverulent 25 lubricant for rendering the metal into particles of spongy form, permeated and coated with the lubricant.

Another object of the invention is to provide a lubricating packing product having 30 a ductile metal base consisting of spongiform metal particles of graded or ungraded dimensions, impregnated and coated with a pulverulent lubricant, adapted to be pressed into form for an article of commerce or as a 35 compound to be applied and compressed into a journal or stuffing box for bearing or packing utility.

Other objects and features of advantages 40 will be more fully revealed in the following detail description of the process and product.

The invention being particularly directed to the production of a metallic packing product having lubricating qualities, the metal 45 or metal alloy as a base, representing any of the commercial or special metal alloys, adaptable for packing or bearing use are herein contemplated, these varying in grade or kind for different classes and degrees of 50 services and having attained a status in the art so as not to require any detailed disclosure herein. Therefore no analytical or formula reference of any alloys will be made.

The desired metal or metal alloy is heated

and while in a molten state, is poured from 55 approximately a height of six feet into a pulverized graphite bath. For the best results the packing metal is heated to a degree bringing the mass to a light cherry red color. The extreme heat of the metal is approximately 2200° Fahrenheit and the heat at 60 pouring point is approximately 950°, varying according to the different alloys used in making different metal alloys. The pulverized graphite is sustained in either a stationary, revolving or moving container. The molten metal, as it strikes the loose graphite, 65 spouts over and imbeds itself into the graphite, converting the cooling metal into cellular or spongy particles permeated and 70 coated with graphite.

Before pouring the molten alloy, any oxide or other foreign accumulation is scraped off of the molten metal. The molten metal can be poured at a different state of fluency from 75 that when heated as described and the product will not be noticeably different except that it will not possess the resiliency desired for some of its uses.

For governing the size of the particles, 80 the molten metal is poured through a screen disposed above the graphite, the screen being preferably disposed at a height of four to eight inches above the graphite. The height from which the molten metal is poured is 85 limited to a distance which will not permit it to cool and assume a permanent shape before striking the graphite.

I am aware that many methods have been practised for producing a metal packing 90 containing graphite, as by mixing graphite into the molten metal or by coating the cold particles of the metal with a graphite, which products, however, are not easily compressible to make an efficient packing or bearing, 95 or, are low in percentage of graphite.

With the product of a spongy or cellulose formation, it is receptive of a high percentage of graphite and the particles will interlock with one another when compressed or 100 moulded into shape, either when preliminarily formed into a gasket or bearing or loosely applied in its place of utilization as in a stuffing-box and compressed within the box about a shaft or stem by the stuffing-box nut 105 or gland. It permits of a larger range of many adjustments in adding to the life of the packing and easily packed to render it im-

pervious to steam at high pressures, as it will not permit hair lines to be blown in it as is common with all other packings. It can be shaped in band or cord form as a flexible strip packing.

Having described my invention, I claim:

1. A process for producing a product of the character set forth, consisting in pouring molten metal alloy from a height upon 10 a quantity of pulverized graphite thereby forming a spongy metal product impregnated and coated with graphite.
2. A process for making a metal packing product, consisting in pouring molten metal 15 from a height upon a quantity of granular lubricant material.
3. A process for making spongy metal products consisting in pouring molten metal

from a height upon a loose pulverized lubricant material.

4. A process for making a lubricating metal packing consisting in pouring molten metal from a height upon loose pulverized graphite.

5. A process for making a lubricating 25 metal packing consisting in pouring molten metal from a height through a screen and upon a loose pulverized graphite.

In witness whereof, I hereunto subscribe my name, as attested by the two subscribing 30 witnesses.

RICHARD F. SPROESSIG.

Witnesses:

L. A. BECK,  
J. C. JUNIUS.